

May 11, 1926.

1,584,607

H. M. BURR

DRINKING CUP AND OTHER RECEPTACLES

Filed Sept. 13, 1923

*Fig. 1.*



*Fig. 2.*



INVENTOR:

*Harry M. Burr*

BY

*Arthur B. Jenkins*

ATTORNEY.

Patented May 11, 1926.

1,584,607

# UNITED STATES PATENT OFFICE.

HARRY M. BURR, OF MIDDLETOWN, CONNECTICUT.

## DRINKING CUP AND OTHER RECEPTACLES.

Application filed September 13, 1923. Serial No 662,368.

My invention relates to that class of receptacles that are commonly made from paper, cloth, or other more or less flexible materials, and which materials are, in their natural state, susceptible more or less to moisture, or that may be readily penetrated by matter in different forms, and an object of my invention, among others, is the production of a receptacle or receptacles that may be made from paper, cloth, or other more or less flexible materials, which receptacle or receptacles may be rendered water-proof and free from the action of heat, and which receptacles shall also be practically free from the penetration of matter of various forms, as, for instance, disease germs.

One form of receptacle embodying my invention and in the construction and use of which the objects herein set out as well as others, may be attained, is illustrated in the accompanying drawings, in which—

Figure 1 is a view in side elevation of a drinking cup embodying my invention.

Figure 2 is a view, scale enlarged, in section through a fragment of the cup, the dimensions as to thickness being greatly exaggerated in order to clearly bring out the invention.

For the purpose of promoting sanitary conditions, it is customary at the present time to provide drinking places with drinking cups of inexpensive construction, such cups being commonly composed of paper and which cups may be discarded immediately after use, and while my invention is not limited in use to a drinking cup, as it is readily adapted for use in such a structure, I have selected such for the purpose of illustration and description of my invention herein.

In the manufacture of drinking cups of the kind and for the purpose above set out, as well as in the construction of various sorts of receptacles and of other devices, to render them sanitary such cups, receptacles and other devices are coated or lined with a material that causes them to be substantially impervious to moisture, disease germs and the like, but such coating material heretofore employed has not been of a nature to withstand heat to any substantial degree.

By the use of my present invention I have provided means whereby various articles, as herein indicated, and especially drinking cups of the paper variety are rendered heat resisting to such extent that heat existing in

liquids will not injure such receptacles, and, further, receptacles lined or coated with my improved coating will be substantially impervious to moisture, disease germs and the like.

In applying my invention a cup 3, or other receptacle or device formed from paper or other flexible material, is treated with one or more coats of my improved coating to be hereinafter described and that possesses requisites as to pliability and flexibility such as not to impair the ordinary use or uses of the devices to which it is applied. This material is also free from absorption or giving off of odors. Such material comprises pyroxyline, or any soluble cellulose material having similar properties, that shall preferably be free from acid, and that is dissolved by the use of a suitable solvent, and that may or may not be mixed with castor oil, that shall also preferably be free from acid. In preparing these ingredients the pyroxyline or cellulose ester is dissolved with high grade wood alcohol or any other solvent, preferably that will leave no odor, and when castor oil is included it will be in a quantity to produce a material having the desired qualities when mixed with a proper quantity of the pyroxyline.

In practicing my invention I have found the following proportions of the pyroxyline, alcohol and castor oil, when the latter is used, to answer satisfactory requirements:

To one part of the pyroxyline or dry soluble cotton, I add five parts of a solvent, as wood alcohol or its equivalent, which are thoroughly mixed, and to this I add one part of castor oil, when the latter is included, that is, in a mixture I have found to be satisfactory I take one hundred pounds of the dry soluble cotton (pyroxyline), five hundred pounds of wood alcohol or other solvent, to which may be added, if desired, one hundred pounds of castor oil.

In application the cup or other receptacle is treated with the solution to a thickness desired, it being preferable to apply the coats at different times, each successive coat being applied after the preceding coat has thoroughly dried. I have found that one to three coats of the mixture will answer all purposes. This provides a coating 4 that may be applied in any desired manner.

After the last coat composed of the ingredient or ingredients above described has been applied I then apply a finishing coat 5

that is composed of pure pyroxyline, this being for the purpose of securing a smooth surface on the object that shall be sufficiently hard to avoid the collection of foreign matter and that shall successively resist heat which may be contained in liquids.

In accordance with the provisions of the patent statutes I have described the principles of operation of my invention, together with the process which I now consider to represent the best embodiment thereof; but

I desire to have it understood that the process described is only illustrative and that the invention may be carried out by other means.

I claim—

15 A drinking cup composed of paper completely covered with a coating composed of a mixture of pyroxylin dissolved in a suitable solvent and castor oil, and an outer coating composed of pure pyroxylin.

HARRY M. BURR.